

July 18, 1944.

K. CLARK ET AL

2,353,879

BOTTLE CAP

Filed Nov. 19, 1940

Fig. 1



Fig. 2



Fig. 3



Fig. 4



INVENTORS  
Kempton Clark  
BY Herbert G. Vore  
Attorney

## UNITED STATES PATENT OFFICE

2,353,879

## BOTTLE CAP

Kempton Clark, Little Compton, R. I., and Herbert G. Vore, Jackson Heights, N. Y., assignors to American Seal-Kap Corporation of Delaware, Wilmington, Del., a corporation of Delaware

Application November 19, 1940, Serial No. 366,218

1 Claim. (Cl. 215—38)

This invention relates to bottle caps and more particularly to a partially preformed hood cap for milk bottles or the like.

An object of the invention is to provide a cap of the above type having novel and improved characteristics.

Another object is to provide a cap of the above type having a thermoplastic adhesive coating of such character that it may be readily heat sealed under conditions encountered in commercial operation.

Another object is to provide a partially preformed cap of the above type which may be readily stacked for shipment and which may be applied to the bottle by standard capping mechanism.

Other objects and advantages will be apparent as the nature of the invention is more fully disclosed.

Although the novel features which are believed to be characteristic of this invention are pointed out more particularly in the claim appended hereto, the invention itself may be better understood by referring to the following description, taken in connection with the accompanying drawing, in which a specific embodiment thereof has been set forth for purposes of illustration.

In the drawing:

Fig. 1 is a perspective view of the partially preformed cap as shipped to the dairy;

Fig. 2 is a top plan view thereof;

Fig. 3 is a side elevation, partly broken away, of the bottle neck and cap, illustrating an intermediate step in the capping and sealing process; and

Fig. 4 is a side elevation, partly broken away, showing the finished cap in place on a milk bottle.

In the following description and in the claim certain specific terms are used for convenience in referring to various details of the invention. These terms, however, are to be given as broad an interpretation as the state of the art will permit.

Referring to the drawing more in detail, the invention is shown as applied to a cap for a standard milk bottle having a neck 10, a pouring lip 11 and an internal ledge 12 adapted to receive a sealing disc or the like.

In accordance with the present invention the cap is made from paper or other fibrous material which is capable of absorbing water and accordingly requires processing to render the same water resistant and which is sufficiently stiff and

rigid to be self-supporting and to possess substantial strength.

The paper blank is first moistened with water so as to render the same pliable for subsequent handling. It is then impregnated with a synthetic thermoplastic resin which is not miscible or soluble in wax and which is capable of being heat sealed at comparatively low temperatures. Examples of materials having the above properties are the following: polyvinyl acetate, polyvinyl chloride, the copolymer of vinyl acetate and vinyl chloride, vinylidene resins and their copolymers, modified glyceryl phthalates known as Rezyls and Rezyl-Balsams, and acrylate resins, either with or without non-toxic plasticizers suited to reduce the sealing temperature thereof. Preferably a resin is used having a sealing temperature below about 200° F. so as to avoid unduly heating the bottle during the sealing operation as well as for ease of application in the dairy.

As a specific embodiment I have found that a polyvinyl resin, such as a suspension of finely divided polyvinyl acetate in an aqueous medium, containing about 60% solids is suitable for the above purpose. The blank, after moistening, may be passed through the suspension and squeezed between rolls to force the same into the paper and to leave a predetermined coating on the surface thereof. This may take place in two stages if desired. In the first stage the rolls may exert a comparatively high pressure on the blanks so as to force a substantial portion of the suspension therein. In the second stage the rolls may exert a lower pressure so as to permit a predetermined coating to remain on the surface of the blank.

The water of the suspension which is thus forced into the blank acts as a plasticizer to assist in maintaining the blank soft and pliable for molding. If sufficient moisture is thus worked into the blank the preliminary moistening step may be omitted. The amount of water in the suspension may be varied to obtain the desired results. A part of the polyvinyl acetate particles in the suspension is also forced into the fibers along with the water and serves to impregnate the outer fibers as well as to form a coating over the surface thereof. The coating is thus firmly bonded to the fibers.

After being coated with the thermoplastic resin as above described, the blank is immersed in a wax bath which may comprise paraffin wax heated to a suitable temperature to maintain the same in a liquid condition. The wax serves to drive

off a part of the water of the suspension and causes the polyvinyl acetate to become partially set. A portion of the water is allowed to remain in the blank, however, so as to maintain the same pliable for molding. The wax also forms a coating on the surface of the blank which prevents the same from sticking together when they are subsequently stacked.

After leaving the wax bath, the blanks are cooled to a sufficiently low temperature for the wax to harden, after which they may be stacked and taken to the forming press.

In the forming press the blanks are partially preformed to provide a central, bore-closing portion 15 adapted to seat within the pouring lip 11 of the bottle 10 on the internal ledge 12 thereof, a U-shaped pouring lip housing 16 joined to the central, bore-closing portion 15 and adapted to cover the pouring lip 11 of the bottle, and a skirt 17. The skirt 17 is formed with a plurality of folds or pleats 18 which extend outwardly beyond the pouring lip housing 16 and are adapted to be folded downwardly around the outer surface of the bottle neck after the cap has been positioned thereon. The preformed pleats 18 are shown as extending outwardly in about the plane of the central bore closing portion 16 but may be extended somewhat downwardly to facilitate the nesting of the caps for shipment and the folding of the skirt about the neck of the bottle.

The wax, together with the moisture in the blanks, serves to maintain the blanks sufficiently pliable for receiving this severe forming operation without tearing the paper. In this condition it is possible to form the pouring lip housing 16 under high pressure so as to form a smooth vertical inner surface 21. The skirt 17 may begin at the top of the outer surface 22 of the pouring lip housing 16 in which case the outer surface is not preformed or a portion of the outer surface 22 above the skirt 17 may be preformed. In any event, the skirt forms a continuation of such outer surface when in place on the bottle. After standing the remaining water is removed by normal evaporation and allows the cap to set in a semi-rigid condition.

A disc 20 may be inserted within the cap either in the forming press or in a subsequent operation so that the cap, as shipped, includes the disc which is securely held therein to form a single unit. The disc may be heat sealed to the blank and thus secured by the thermoplastic adhesive or may be held in place by the friction of the side walls of the pouring lip housing. The caps partially preformed, as above described, may be stacked and shipped to the dairy.

At the dairy the caps are applied to the bottle by a suitable capping head which forces the bore closing portion 15 within the bottle neck and folds the pleated skirt downwardly about the outer surface of the pouring lip, as shown in Figs. 3 and 4. Heat and pressure is then brought to bear upon the folded pleats for rendering the thermoplastic material tacky and causing the pleats to permanently adhere together when the material has again cooled. It is usually desirable to maintain the pressure until the material has cooled to a point such that adhesion is attained.

In the above described process, the wax coating, in addition to drying and partially setting the polyvinyl acetate, is absorbed within the fibers around the edges of the blank where the susceptibility is the greatest and also at any points on the surface of the blank where the

resin coating may be incomplete, and thereby increases the water resistance of the blank. The resin coating may be varied so as to provide a substantially wax-free blank or to allow a predetermined amount of wax to be absorbed therein as desired. The blank may thus be partially impregnated with both wax and resin. Under heat and pressure the wax coating softens and exposes the resin so that the resin coatings of the pleats come into surface contact for sealing.

10 A small amount of an anti-oxidant may be added to the paraffin wax bath so as to prevent the bath from oxidizing. The polyvinyl acetate may include a suitable plasticizer so as to render the same heat sealable at temperatures below 200° F. It is usually undesirable to heat the cap when in place on a milk bottle to temperatures greatly above this value. The milk bottle, being cold, readily cools the cap after the heating step and facilitates the setting of the thermoplastic resin.

15 In certain instances a suitable binding agent, such as aluminum acetate, may be added to the polyvinyl acetate suspension so as to effect a more complete bond with the paper. Such an agent may be present, for example, in a small proportion such as about 5%. Other materials, such as isomerized rubber (Pliolite), chlorinated rubber, paracumarone-indene resins, cellulose esters, terpene resins, polybutene or other materials which can be made into a water suspension 20 or emulsion or otherwise incorporated in the polyvinyl acetate suspension may be added 25 and facilitates the setting of the thermoplastic resin.

25 In certain instances a suitable binding agent, such as aluminum acetate, may be added to the polyvinyl acetate suspension so as to effect a more complete bond with the paper. Such an agent may be present, for example, in a small proportion such as about 5%. Other materials, such as isomerized rubber (Pliolite), chlorinated rubber, paracumarone-indene resins, cellulose esters, terpene resins, polybutene or other materials which can be made into a water suspension 30 or emulsion or otherwise incorporated in the polyvinyl acetate suspension may be added 30 and facilitates the setting of the thermoplastic resin.

35 35 Although the above described coating is present on both sides of the blank, nevertheless, the nature of the coating is such that it does not adhere to the bottle. The cap is accordingly 40 sealed in place solely by the adherence of the pleats of the skirt to themselves. Hence the cap may be removed without fouling the bottle by merely tearing the same or by breaking the seal between the pleats. In any event, the cap cannot be re-applied and re-sealed without showing 45 on inspection that the cap has been previously removed.

40 Obviously, the thermoplastic adhesive coating may be applied to only one side of the blank, if desired, preferably to the side forming the outside of the finished cap. The wax may then be applied to both sides as above described or may be applied only to the uncoated side of the blank.

45 In certain instances it may be desirable to omit the disc 20. However, the disc is usually preferred in order to increase the frictional engagement between the wall of the cap and the inner surface of the pouring lip of the bottle and to assist in holding the cap in place. The use of a disc 20, as shown, permits the cap to be formed from thinner paper than would otherwise be required and thereby decreases the cost of manufacture. The use of thin paper also increases the ease of sealing the pleats together.

50 55 The above described cap constitutes, in effect, a hood cap which covers the pouring lip of the bottle. The cap is formed as a single unit which includes the hood and the disc so that only a single operation is required in capping the bottle. Furthermore, the cap and disc are removed as a unit and in a single operation. The cap is accordingly sanitary, tamper-proof and convenient for the consumer. The wax and resin render the cap moisture proof so that it is not affected by 60 normal conditions of use.

It is to be understood that polyvinyl acetate is referred to merely as an example of a synthetic resin having the characteristics required for the above purpose. Other synthetic resins having similar properties and having non-toxic characteristics may also be used.

Although a specific embodiment of the invention has been shown for purposes of illustration, it is to be understood that various changes and modifications may be made therein as will be readily apparent to a person skilled in the art. The invention is only to be limited in accordance with the scope of the following claim.

What is claimed is:

A milk bottle cap formed from a paper blank, 15

said cap comprising a bore closing portion and a pleated skirt extending downwardly around the outer surface of the pouring lip of the bottle, at least the skirt portion having a coating of a thermoplastic adhesive suited to secure the folds together comprising essentially polyvinyl acetate which becomes tacky for sealing at a temperature below about 200° F. and which is set at room temperature, and a wax coating over said adhesive to prevent the caps from sticking together when stacked, said coating being adapted to be displaced to expose the adhesive under sealing conditions of heat and pressure.

KEMPTON CLARK.  
HERBERT G. VORE.